

Oct. 10, 1950

E. L. SCHULMAN

2,524,932

PROCESS FOR PRODUCING BONDED MICA

Filed Sept. 12, 1946

Fig. 1.



Fig. 2.



Fig. 3.



WITNESSES:

E. G. McElroy  
Jew. L. Groome

INVENTOR

Earl L. Schulman.  
BY  
Frederick Shapoe  
ATTORNEY



Fig. 3 is a schematic view of a process for producing formed mica insulation.

According to the present invention layers or bodies of mica flakes treated with a fluid or a flowable binder are subjected to a substantially uniform unit pressure over the entire surface thereof. More specifically, the body of mica flakes and flowable binder applied thereto is subjected to pressure applied through an elastic member, said elastic member being subjected to fluid pressure. The elastic member will conform to and apply a substantially uniform pressure regardless of the shape or form of the surface of the mica body to which it is applied.

Referring to Fig. 1 of the drawing, there is illustrated an apparatus 10 for carrying out the process. The apparatus comprises a substantially rigid platen or base 12 provided with hollow coils or tubes 14 in which a heating fluid or a cooling fluid may be circulated to secure predetermined temperatures. It will be appreciated that the tubes 14 may contain an electrical heating element or other heating means if desired. Disposed above the platen 12 is a movable press head 16 having a cavity 18 disposed along its underside. An elastic member 20 is applied to the head 16 to close the cavity 18. A conduit 22 is disposed in the head 16 for introducing steam or hot water or other suitable fluid under pressure into the cavity 18. Cooling water may be introduced into the cavity by the conduit 24 and vented through the conduit 26. The elastic member or diaphragm 20 may be secured to the sides of the press head 16 by means of bands or clamps 28. The elastic member 20 is preferably an elastomer, such as rubber or polychlorobutadiene or a silicone polymer, commonly known as "silastic," capable of withstanding elevated temperatures.

A layer of mica flakes 30 may be prepared in a conventional mica laying machine wherein mica flakes are dropped upon a moving screen from an overhead distributor and disposed as a more or less uniform layer and thereafter a suitable binder is applied thereto by dripping, sprinkling or the like. The mica flake layer 30 is subjected to a preliminary heating with or without vacuum treatment to remove essentially all the volatile solvent from the binder prior to being placed in the apparatus 10. The uncompacted layer of mica flakes with the binder distributed therein will be found to be heterogeneously disposed and characterized by relatively high spots and low spots due to natural variation in distribution. Hand laid sheets may be somewhat more uniform but are still subject to unavoidable irregularities so that relatively high and low spots are present.

The fluid binder is preferably, though not necessarily, a heat curable or thermosetting composition. Examples of such compositions are shellac, mixtures of shellac with gum elemi or copal gum or other natural resin, alkyd resins, or alkyd resins combined with a vinyl or vinylidene monomer, and other resinous compositions. In some cases, inorganic compositions capable of curing to a relatively thermoset state may have been applied to the mica flakes. Solutions of the binder in a volatile solvent are commonly employed. After heat treatment to remove the solvent, the binder in the mica layer is not a true fluid composition but is capable of fluid flow when heated and pressure is applied thereto.

The mica layer 30 with the uncured flowable binder is placed on the flat platen 12, as shown in Fig. 1, and is subjected to consolidation by moving the head 16 until the diaphragm 20 is in

contact with the upper surface of the mica layer 30 and fixing the head in this position. Steam is then admitted at a pressure of from about 20 to 100 pounds per square inch through the conduit 22, thereby forcing the elastic member 20 at a corresponding unit pressure against the upper surface of the mica layer. Heat from the steam is transferred through the elastic member to the mica layer 30. Simultaneously, steam or hot water may be admitted to the tubes 14 in the platen 12 for heating the layer of mica flakes from the underside. Through the agency of the elastic member the fluid pressure is distributed substantially uniformly over the entire layer 30 regardless of high or low spots in the layer. The high spots will not be subjected to crushing nor will they be subject to unit pressures differing from the unit pressure at low spots and there will be no tendency to drive the binder to lower spots. Therefore, the binder will be substantially uniformly distributed with respect to the mica throughout the entire layer 30. Pools or puddles of binder will not form at any point. The pressure and heating may be continued for a period of time of from a few minutes to one hour or more. With heat curable binders the temperature selected and the time of application of heating and pressing will be selected in accordance with the type of product desired. A fully cured product may be desired in some cases and temperatures of as much as 700° C. and times of one hour for the treatment may be employed. Where a partially cured sheet of mica composition is desired, for example, for reforming into some complex shape, the treatment may be carried out only for a few minutes.

At the end of the predetermined pressing period, the admission of steam or hot water to the conduit 22 is terminated and cooling water or the like will be admitted to the conduit 24. The cooling water after circulation in the cavity 18 may be vented through the conduit 26 until the mica insulation has been cooled down to room temperature or thereabouts. The press head 16 is then elevated and the mica layer 30 removed from the press.

Referring to Fig. 2 of the drawing, there is illustrated a cross section through the layer of bonded mica 30 resulting from the pressing operation. The lower surface 34 of the mica will be flat due to contact with the upper surface of platen 12. The upper surface 36 of the mica layer will be extremely rough in appearance, though an examination of the mica sheet against the light will show an exceptional degree of transparency which is not possessed of by any mica material of equal thickness using the same binder as produced by any conventional process known. It will be apparent, however, that for most applications the rough upper surface 36 must be removed by machining to the level shown as 32 to produce a sheet of substantially uniform thickness with a smooth upper surface. It will be found that the product produced by the apparatus of Fig. 1 must be machined considerably more to secure a perfectly flat sheet than the mica compositions of the prior art. This is due to the fact that prior art processes tended to drive the binder into the low spots of the layer, thus building up the low spots and crushing the high spots, thereby attaining a lesser degree of non-uniformity of the upper surface 36 at the expense, however, of the uniformity of distribution of binder and the integrity of the mica itself. For a given size sheet, it is necessary to

press 25 to 26 ounces of mica to secure a level 10 mil thick sheet by the process of the present invention, whereas prior art presses employing a felt pad require only 19 ounces of mica for the same thickness of sheet. However, the uniformly thick sheet produced by the machining operation of the present invention is incomparably better both electrically and mechanically than the prior art mica laminate.

As a specific example of the practice of the invention, a sheet of 25 ounces of 6-1st splittings of mica was treated with 20% alcoholic solution of shellac until approximately 2½ ounces of shellac solids had been applied thereto. The ratio of shellac to mica was 1 to 10. The sheet was thoroughly dried in the oven at 80° C. for 10 minutes to evaporate the alcoholic solvent to an amount of less than 0.1%. The sheet was pressed in a press similar to that of Fig. 1 using steam at 40 pounds per square inch and a temperature of 140° C. for 8 minutes. Therefore, the steam was shut off and cooling water admitted for 6 minutes. The cooling water was applied under a pressure of 45 pounds per square inch. The sheet was machined by means of a sanding drum to a thickness of 0.01". Another sheet of mica was prepared in a similar way employing 19 ounces of mica with sufficient alcoholic flake solution applied to provide 1.9 ounces of shellac thereto and pressing in a hydraulic press employing the best known process of the prior art using a board ½" thick composed of cotton and felt between the press head and the mica layer. The temperatures and pressures employed were similar to those applied to the former sheet, except that the pressure was averaged over the entire layer in the latter case. After machining to a thickness of 0.01", the sheet was cut into 1" squares. The amount of the shellac binder in each of 25 1" squares selected at random was determined by analysis. The sheet produced in the apparatus of Fig. 1 was similarly cut up in 1" squares and the binder content determined for each of 25 1" squares. The bond content of the squares of mica produced in accordance with this invention varied from 8% to 11.8%, whereas the bond content of the mica produced by means of a felt pad only varied from 8% to 16.8%. The coefficient of dispersion for the bond content was 20.7% for the sheet produced by prior art practice and 10.8% for the sheet produced according to the present invention. A comparison of the compressibility at 1000 pounds per square inch and a temperature of 150° C. showed that the sheet of the present invention had a compression set of 1.00% whereas that produced by using the felt pad was 1.37%. Examination of the mica composition produced in accordance with this invention showed no crushed spots, whereas that produced by means of the felt pad showed crushed mica in several places.

The mica compositions of this invention have substantially greater density than those produced by any prior art process. Members of identical size and shape weighed from 1 pound 8 ounces to 1 pound 9 ounces for the pad pressed member and the hydraulically pressed member weighed from 1 pound 10 ounces to 1 pound 11 ounces. The average density was approximately 8% higher for mica produced according to the present invention. This is reflected in superior properties all out of proportion to the increase in density.

In consolidating mica by pressure and heat treatment in the apparatus of Fig. 1, for example, the binder in the mica layer 30 may be cured suf-

5  
10  
15  
20  
25  
30  
35  
40  
45  
50  
55  
60  
65  
70  
75

ciently to be substantially free of fluid flow but not completely heat cured to a relatively thermoset condition. For shellac this corresponds to 4 or 5 minutes at 130° C. The partially cured sheet 30 may be further processed into shapes other than flat sheets by the process schematically shown in Fig. 3 of the drawing. After having been pressed to a partially cured state at 10, the sheet of mica 30 is placed on a support 40 and machined by the sanding drum, milling cutter or other suitable implement 42 to remove the rough top surface 36 shown in Fig. 2 of the drawing. A relatively smooth upper surface will be produced. It will be appreciated that the machined upper surface will ordinarily be parallel to the bottom surface 34 of the pressed mica sheet. However, in some cases the sheet of mica may be machined at an angle to the bottom or in some other form in accordance with the requirements of the particular application. Thereafter the machined mica 30 may be formed to some other shape such, for example, as a V ring. To accomplish this, the machined sheet of mica is placed in a heated die 44 provided with a V groove 46 and pressed by the moving head 48 provided with a V 50. The V 50 may be heated when subjected to temperatures of 100° C. to 150° C. or even higher, for one hour the binder in the mica sheet will cure completely and upon release of pressure a permanently set V ring 60 will be then obtained.

V rings produced from mica sheets formed in accordance with the process of this invention have been compared with those produced by conventional processes and have been found to be superior both electrically and mechanically due to the absence of crushed spots and due to the more uniform distribution of binder in the V ring.

It will be appreciated that the times and temperatures and pressures set forth herein are only exemplary and in each case a proper selection must be made depending upon the type of resinous binder employed. Some resinous compositions cure fully at moderate temperatures and pressures in a short time such, for example, as a solution composed of 60% monostyrene and 40% of the reaction product of maleic anhydride and glycol, while other resins, for example, shellac may require much longer periods of time and elevated temperatures.

While the apparatus of Fig. 1 has been shown to comprise a relatively stationary platen 12 and a movable press head 16, the movement of the parts may be reversed so that the platen 12 may be the movable member. Furthermore, a plurality of platens and press heads each provided with an elastic member may be employed in a single press. Likewise the upper surface of the platen 12 may be of some other shape than the plane surface indicated in the drawing. For most applications, however, the upper surface of the platen 12 is preferably a plane. As is well known in the art, a layer of paper, cellophane, a metal screen, or a parting compound may be placed on the surface of the platen 12 to facilitate removal of the pressed layer of mica after treatment.

While excellent results have been obtained by consolidating mica flakes with a binder by compressing the mica by means of hydraulic pressure applied through an elastic diaphragm, a product of similar quality has been prepared in another manner. In this latter case a highly resilient elastomeric blanket about ½ inch to 1 inch or thicker may be placed between one face of the press platen and the mica body being consolidated.

The following resilient elastomeric materials have been found successful: natural rubber, sponge rubber, silicone rubber and neoprene. The elastomeric material must be sufficiently thick and resilient as to flow and thereby redistribute the unit pressure to substantially the same value at the mica face. The following table gives the coefficient of dispersion of a shellac bond in a 10 mil thick sheet of bonded mica prepared initially with 10% by weight of shellac based on the weight of the mica:

|                                                                                      | Per cent |
|--------------------------------------------------------------------------------------|----------|
| Hydraulically pressed                                                                | 10.8     |
| Conventional pressed— $\frac{1}{8}$ " asbestos pad                                   | 21       |
| Conventional pressed—no pad                                                          | 19       |
| Conventional press— $\frac{1}{8}$ " thick rubber blanket of 60 Shore A hardness      | 89       |
| Conventional press— $\frac{1}{2}$ " thick rubber blanket of 50 Shore A hardness      | 90       |
| Conventional press— $\frac{3}{8}$ " thick sponge rubber blanket of 15 Shore hardness | 13.2     |
| Conventional press— $\frac{1}{2}$ " thick rubber blanket of 50 Shore hardness        | 11       |

It will be noted that the asbestos pad gives a coefficient of dispersion about the same as that obtained with no pad. This indicates that the high spots are almost equally over pressed.

The  $\frac{1}{2}$ " and  $\frac{3}{8}$ " thick rubber blankets are so thin that they crush almost completely without any substantial flow and this impairs the bond distribution. Therefore, a thin rubber blanket is a detriment rather than a benefit in pressing mica.

The use of an elastomeric pressing blanket of  $\frac{3}{8}$ " thick or thicker gives results entirely unexpected in view of the negative results obtained from both the  $\frac{1}{2}$ " and  $\frac{3}{8}$ " rubber blanket. It is thought that an elastomeric blanket about  $\frac{3}{8}$ " thick is required to secure sufficient body to secure a true flow of the elastomer thereby rendering the unit pressure constant.

The process of this invention is most advantageous for treating mica combined with a heat curable binder which may well be reacted to a relatively thermostat state. The use of hydraulic pressure applied through an elastic membrane also may be beneficial in consolidating mica sheets treated with a thermoplastic binder. In the latter case consolidation will produce a well bonded mica sheet having no crushed mica and free from undesirable bond distribution.

Since certain obvious changes may be made in the above procedure and different embodiments of the invention could be made without departing from the scope thereof, it is intended that all matter contained in the above description shall be interpreted as illustrative and not in a limiting sense.

I claim as my invention:

1. In the process of preparing bonded mica, the steps comprising placing a sheet of mica flakes carrying a heat curable flowable binder on a relatively rigid, smooth base, covering the sheet of mica flakes with an elastic member, forcing the elastic member against the sheet of mica flakes in the direction of the base by means of fluid pressure thereby to apply a uniform pressure and to secure a uniform distribution of the binder relative to the mica, heating the sheet of mica flakes at a temperature sufficient to cure the binder to a non-flowable state, removing the heat cured mica sheet from the base and machining to smoothness the relatively rough surface that

has resulted from contact with the elastic member.

2. In the process of preparing bonded mica, the steps comprising placing a sheet of mica flakes carrying a heat curable, flowable binder on a relatively rigid, smooth base, covering the sheet of mica flakes with an elastic member, forcing the elastic member against the sheet of mica flakes in the direction of the base by means of fluid pressure thereby to apply a uniform pressure and to secure a uniform distribution of the binder relative to the mica, heating the sheet of mica flakes at a temperature sufficient to cure the binder, continuing the application of heat and pressure until the binder is partially cured sufficiently to be substantially free of fluid flow, removing the partially heat cured mica sheet from the platen, machining to smoothness the relatively rough surface that has resulted from contact with the elastic member, and reforming the partially cured mica sheet under heat and pressure to predetermined shape until the binder is fully cured to a non-flowable state.

25 3. In the process of preparing bonded mica insulation, the steps comprising forming a body of mica flakes and a heat-curable flowable binder applied thereto, subjecting the formed body to substantially the same pressure over the entire surface while being heated at an elevated temperature suitable for curing the binder, thereby providing a uniform distribution of the binder throughout the compressed body, continuing the application of heat and pressure until the binder is cured to a non-flowable state, and machining the relatively rough surface of the bonded mica product so produced to remove surface irregularities.

4. In the process of preparing bonded mica insulation, the steps comprising forming a body of mica flakes and a heat-curable flowable binder applied thereto, disposing a blanket of a resilient elastomer at least about  $\frac{1}{8}$  inch thick upon the body, placing the body and applied blanket into a press, subjecting the formed body to substantially the same pressure over the entire surface while being heated at an elevated temperature suitable for curing the binder, thereby providing a uniform distribution of the binder throughout the compressed body, continuing the application of heat and pressure until the binder is cured to a non-flowable state, and machining the relatively rough surface of the bonded mica product so produced to remove surface irregularities.

5. In the process of consolidating a layer of mica with an applied hardenable binder disposed on a smooth, unyielding base, the step comprising subjecting the layer of mica flakes and the binder applied thereto to a substantially uniform unit pressure over the entire layer whereby the binder is substantially uniformly distributed with respect to the mica flakes, hardening the binder, and machining irregularities off the surface of the mica layer that was not against the smooth base.

6. In the process of consolidating a layer of mica with an applied heat curable binder disposed on a smooth unyielding base, the step comprising applying fluid pressure through an elastic member to the layer of mica flakes and the applied binder distributed within the layer to consolidate the layer of mica flakes and binder with the binder being substantially uniformly distributed in the layer, heat curing the binder, and machining irregularities off the surface of the

mica layer that was not against the smooth base.

7. In the process of producing bonded mica, the steps comprising preparing a layer of mica flakes and a flowable thermosettable binder distributed therein, compressing the layer between a relatively rigid flat smooth surface and a yielding resilient surface corresponding in its effect to a fluid diaphragm member, to apply to the layer a substantially uniform pressure over the entire surface of the layer at a value below that sufficient to crush mica flakes, whereby a substantially uniform distribution of the flowable binder with respect to the mica flakes is produced, heating the compressed layer to a temperature sufficient to thermoset the binder, relieving the pressure on the layer thereby producing a bonded mica layer having one flat, smooth surface and the other surface being highly irregular with many projections, and machining the irregular

surface to remove the projections whereby a bonded mica layer of great uniformity in physical and electrical properties is obtained.

EARL L. SCHULMAN.

#### REFERENCES CITED

The following references are of record in the file of this patent:

#### UNITED STATES PATENTS

| Number       | Name     | Date           |
|--------------|----------|----------------|
| 1,776,885    | Cheetham | Sept. 30, 1930 |
| 2,012,948    | Boughton | Sept. 3, 1935  |
| 2,057,672    | Ellis    | Oct. 20, 1936  |
| 15 2,195,254 | Miller   | Mar. 26, 1940  |
| 2,401,299    | Glavin   | June 4, 1946   |
| 2,420,172    | Griffeth | May 6, 1947    |
| 2,454,210    | Runk     | Nov. 16, 1948  |